

Aug. 17, 1943.

G. H. VON FUCHS

2,327,158

PROCESS FOR PREPARING LUBRICATING OILS

Filed March 3, 1941



Inventors: George Hugo von Fuchs  
Hyman Diamond

By their Attorney: S. W. Luebke

## UNITED STATES PATENT OFFICE

2,327,158

## PROCESS FOR PREPARING LUBRICATING OILS

George Hugo von Fuehs and Hyman Diamond,  
Alton, Ill., assignors to Shell Development Company,  
San Francisco, Calif., a corporation of  
Delaware

Application March 3, 1941, Serial No. 381,530

9 Claims. (Cl. 196—34)

This invention relates to a new method for processing mineral oils to produce lubricating oils of high stability, and more particularly deals with a method wherein lubricating oil stocks are fractionated and reblended according to a novel procedure.

The main purpose of this invention is to fractionate mineral lubricating oil stocks in a manner so that on reblending the several fractions, not only the viscosity of the blend can be controlled but within limits its oxidation stability as well.

It is common practice in the manufacture of lubricating oils to divide available lubricating oil stocks by fractional distillation into so-called neutral oils and bright stocks, i. e., residual oils, and thereafter producing oils of different viscosities by blending two or more of these fractions with each other in the necessary proportions to obtain whatever viscosity may be desirable. Thus relatively light oils as the SAE 10 and 20 grades normally comprise predominating amounts or consist of neutral oils, while the heavier grades contain as a rule more bright stock.

Now we have discovered that lubricating oils of different viscosities produced by blending given neutrals and bright stocks in different proportions have different oxidation stabilities. In the case of well-refined oils we have found that as a rule intermediate-viscosity grades containing substantial portions of both neutrals and bright stocks, have the highest stabilities. We have concluded that the reason for this peculiar behavior is caused by a component which is normally contained in bright stocks in varying amounts, namely, the bright stock resins. Bright stock resins as herein defined are high-boiling normal constituents of bright stocks. They are recognized by their ability of being adsorbed by silica gel and other acid solid adsorbents but are less readily adsorbed by alkaline or non-acidic adsorbents such as fuller's earth, bauxite, zeolites, etc.

It has been known for some time that high-boiling mineral oils contain resins, and that an approximate analytical method for determining their content has been described by Kalichevsky and Fulton in National Petroleum News, volume 23, Number 51, pages 33-6, 1931. It was heretofore generally believed that these resins form a more or less undesirable portion of lubricating oils being responsible for high carbon residue of lubricating oils. Therefore, considerable efforts have been expended in the past to find methods

for deresining lubricating oils, in the hope of thereby reducing carbon residues. However, apparently it remained unnoticed that these resins have a very strong influence on the oxidation stabilities of the oils, which influence may be beneficial or detrimental depending upon the concentration of the resins in the oil and on the susceptibility of the particular oil to the resins.

We have definitely established that any well-refined mineral lubricating oil should contain a certain amount of resins for maximum stability. What this amount should be cannot be stated in general terms because of several difficulties. In the first place, it appears that the group of substances known as resins is rather complex and apparently contains components some of which are effective in smaller concentrations than others. Moreover, in the usual processes of isolating or concentrating resins, resin concentrates are obtained which besides the resins normally contain harmful impurities. These impurities actually may cause a decrease in the stability of blends containing otherwise an optimum quantity of the beneficial resins. Again different oils have vastly different susceptibilities towards the resins. Thus some oils may tolerate or necessitate relatively large amounts of resins, while others reach their maximum stabilities at much lower concentrations. A further difficulty resides in the inaccuracy of the analytical method, which not only fails to give close checks between duplicate determinations, but also fails to distinguish between the useful resins and certain inert or harmful impurities which normally are associated with the former.

In view of the above, the only practical way of determining the optimum concentration of resins in any one oil is to add successively larger amounts of resins to different samples of this oil and then determine the oxidation stability of the several blends so obtained by any of the accepted oxidation methods, preferably in the presence of iron. By plotting the stabilities so obtained against the amount of resins or resin concentrate added, the optimum blend is then easily established.

Having once recognized that the presence of resins in limited amounts in lubricating oils has definite advantages, our procedure of controlling both the viscosities and the stabilities of lubricating oils, resolves itself into producing besides the conventional neutral oils at least two high viscosity stocks, one of which is a bright stock of low resin content and the other is a resin concentrate. Our improved oils are then produced

by blending an amount of resin concentrate with low-resin content bright stock and the neutrals so as to give a blend having the approximate desired viscosity, which amount is such as to result in maximum oxidation stability. If the oils to be produced are very light, e. g., of the SAE 10 grade, the blend may consist of neutral oil and resin concentrate only. Heavier grades are normally produced by blending neutral oil, low resin content bright stock and resin concentrate in suitable proportions.

While, as previously pointed out, the most desirable amount of resins to be added cannot be predicted but must be established experimentally for lubricating oils from different sources, we find that the optimum resin contents normally vary between about 1% to 10%, and more often than not between about 3% and 7%.

Bright stocks of low resin content and resin concentrates are most readily obtained by treating conventional bright stocks such as properly deasphalted (and dewaxed, if necessary) heavy mineral oil distillation residues with normally gaseous hydrocarbons at elevated pressures, preferably at pressures and temperatures near or above the critical conditions of these light hydrocarbons. These conditions are known as para-critical conditions.

The operation of deresining is well known in the art of lubricating oil manufacture. Two fractions are thereby obtained, a bright stock of low resin content and a resin concentrate. As a rule, both the deresined bright stock and the resin concentrate have lower oxidation stabilities than the bright stock from which they are derived.

Bright stocks from which the resin concentrates are obtainable may be produced by any conventional method of manufacture, such as topping a crude petroleum oil containing lubricating oil stock to produce a residue having a suitable viscosity and removing asphalts (and waxes, if necessary) as by propane precipitation or other known means. Vacuum-distilled heavy oils normally yield relatively small amounts of resins. In fact the natural resin content of such oils is normally lower than is required for optimum stability. They may, however, be used in place of the low-resin bright stock in making up blends.

The effectiveness of the resins as oxidation stabilizers may be considerably improved by removing therefrom certain impurities which are normally associated therewith. We have discovered that harmful impurities can effectively be separated from the desirable resins by treating the precipitated resin mixture or the resin concentrate with a neutral or alkaline-reacting adsorbent such as bauxite, brucite, basic permutites, naturally active decolorizing clays as Florida clay and Attapulgus clay, fuller's earth, etc. These adsorbents peculiarly enough are selective for many of the impurities normally associated with the resins, but do not adsorb to any great extent the resins themselves. Therefore in our preferred procedure we treat the resin concentrate preferably in solution in a low-boiling hydrocarbon oil such as naphtha, kerosene, etc., with a neutral- or basic-reacting mineral adsorbent, prior to blending it with a low-resin content lubricating oil.

Strong sulfuric acid in sufficient amounts attacks both impurities and desirable resins. Therefore the resin concentrate cannot be purified by acid treatment. Moreover, because resins

are susceptible to attack by sulfuric acid, it is not desirable to treat bright stocks from which resins are to be separated, with excessive amounts of sulfuric acid. If for some reason severe acid treatment of the bright stock is desired, this should be carried out after the resins have been separated to avoid their being destroyed.

In order to illustrate our invention, reference is had to the attached drawing which represents a graph wherein concentration of resins in various lubricating oils of about the same viscosities is plotted against oxidation stability as measured by the time required to absorb 1800 cc. of oxygen per 100 grams of oil by contacting the oil under standardized conditions with oxygen in the presence of iron (temperature 313° F., 5 sq. cm. exposed iron surface per gram of oil, oxygen pressure 760 mm. Hg). The oils were prepared by blending a (1) resin-free bright stock, (2) a neutral oil and (3) resins, to produce mixtures containing 50% neutral and 50% mixed bright stock and resins, the ratio of bright stock to resins being different in the several mixtures. As will be seen from the drawing, a maximum stability is indicated at a resin content of about 5%.

Concerning the effects of impurities contained in resins, the following data are significant: A heavy lubricating oil containing untreated resins had an oxidation stability of 620 minutes measured as described above. After contacting this oil with fuller's earth once, the stability rose to 890 minutes. Contacting the oil two additional times with fuller's earth raised the stability to 1600 minutes. Now when contacting this very stable oil once with silica gel, the stability dropped to 1000 minutes, and upon further contacting it two additional times with silica gel, it fell to 890 minutes.

We claim as our invention:

1. Process for manufacturing lubricating oils comprising producing at least one low resin content mineral lubricating oil and a petroleum resin concentrate, purifying the latter without materially altering the resin content, and blending said low resin content oil with the purified resin concentrate, in an approximate proportion to produce a blend containing between 3 and 7% resin and having about maximum oxidation stability.

2. Process for manufacturing lubricating oils comprising producing at least one low resin content mineral oil and a petroleum resin concentrate, contacting the latter with a basic reacting mineral adsorbent whereby acidic impurities are adsorbed without materially altering the resin content, and blending said low resin content oil with the contacted resin concentrate in an approximate proportion to produce a blend containing between 3 and 7% resin and having about maximum oxidation stability.

3. The process of claim 2 wherein said adsorbent is bauxite.

4. Process for manufacturing lubricating oil comprising producing at least one low resin content mineral lubricating oil and a petroleum resin concentrate, separately subjecting said low resin content oil to a refining treatment to improve its oxidation stability, contacting said resin concentrate with a basic reacting mineral adsorbent whereby acidic impurities are adsorbed without materially altering the resin content, and blending the treated low resin oil with the contacted resin concentrate in an approximate

proportion to produce a blend containing between 3 and 7% resin and having about maximum oxidation stability.

5. The process of claim 4 wherein said refining treatment of the low-resin content oil comprises sulfuric acid treatment.

6. Process for manufacturing lubricating oils comprising producing three oil components, a neutral oil, a petroleum low-resin content bright stock and a resin concentrate, purifying the latter without materially altering the resin content, and blending said three components to produce a blended oil of predetermined viscosity containing an amount of resins which results in maximum oxidation resistance the amount of resin in said blend being between 3 and 7%.

7. Process for manufacturing lubricating oil comprising subjecting a deasphalted residual lubricating oil stock of low wax content to a 20 deresining treatment to produce a bright stock of lower resin content and a resin concentrate, purifying the latter without materially altering the resin content, and blending said bright stock with at least one neutral oil and said resin concentrate in approximate proportions to produce 25

a blend of about maximum oxidation resistance the amount of resin in said blend being between 3 and 7%.

8. The process of claim 7 wherein said deresining treatment comprises treating the residual stock with a normally gaseous hydrocarbon under para-critical conditions of said hydrocarbon.

9. Process for manufacturing lubricating oils comprising subjecting a deasphalted residual lubricating stock of low wax content to a 10 deresining treatment to produce a bright stock of low resin content and a resin concentrate, separately subjecting said bright stock to a refining treatment capable of improving its oxidation 15 stability, contacting said resin concentrate with a basic reacting mineral adsorbent whereby acidic impurities are adsorbed without materially altering the resin content, and blending the resulting refined low resin bright stock with at least one neutral oil and with the contacted resin concentrate in approximate proportions to produce a blend containing 3 and 7% resin and having about maximum oxidation stability.

GEORGE HUGO VON FUCHS.  
HYMAN DIAMOND.